

June 7, 1932.

J. C. McFARLAND

**1,862,231**

## DECORATING BASE METALS OR ALLOYS OF BASE METALS

Filed June 22, 1928



Inventor:  
James C. McFarland,  
By Dreyfus, D. C. Ritter, of Phila.  
Attys.

## UNITED STATES PATENT OFFICE

JAMES C. MCFARLAND, OF FORT THOMAS, KENTUCKY, ASSIGNOR TO THE WADSWORTH WATCH CASE CO., OF DAYTON, KENTUCKY, A CORPORATION OF KENTUCKY

## DECORATING BASE METALS OR ALLOYS OF BASE METALS

Application filed June 22, 1928. Serial No. 287,536.

The present invention relates particularly to a process for decorating base metals by means of contrasting metal platings, and is in the nature of a modification of the process described in application, Serial No. 287,535, filed of even date herewith.

The primary object is to provide a very simple and effective method of decorating metals by means of platings of contrasting colors.

The process is well adapted to the purpose of decorating movement blocks, for example, employed in watches. Such a block may be composed of any suitable metal, such as what is known on the market as 12% nickel. The composition just referred to is composed of about 12% nickel, 70% copper, and 18% zinc. The process is applicable to other metals, or alloys of metals, however.

The process is illustrated in the accompanying drawing, in which—

Fig. 1 illustrates a base plate having a resist design applied thereto; Fig. 2 illustrates a further step in which chromium plating is applied to the exposed areas of the base plate; Fig. 3 illustrates a further step in which the resist design has been removed, leaving exposed areas of the original surface and leaving the chromium plating design; Fig. 3A illustrates a further step in which the exposed areas of the base plate are etched; and Fig. 4 illustrates a further step in which the exposed areas have been plated with a platable metal which is insoluble in ferric chloride, such as the precious metals or alloys thereof.

In the illustration given in the drawing, A designates a base plate which may be composed of a base metal, or an alloy of base metals; B designates a resist design applied to the surface of the base plate; C designates a chromium plating design applied to the exposed areas of the base plate; A' designates exposed areas of the base plate produced by removing the resist; A<sup>2</sup> designates etching on the exposed areas of the base plate; and D designates a precious metal plating design applied to the exposed areas of the base plate.

The surface of the plate, or body A, may

be of any desired cross-sectional contour, and may be polished, or pumiced, if desired.

The resist design may be applied in any desired manner. Preferably, it is applied by means of a photographic process, such as the one described in Beebe and Murray Patent 1,574,357, granted February 23, 1926.

In accordance with the method there described, a light-sensitive coating is applied to the original metal surface, and an image is produced in the sensitive coating photographically, or by means of light transmitted through a transparency bearing a suitable design; and the unreacted portions of the sensitive coating are then removed by a suitable developing operation, leaving upon the surface the reacted portions of the film in the form of the desired design.

The exposed areas of the original surface are now plated with a chromium plating; the resist design is then removed by means of a suitable solvent, leaving exposed areas of the original surface and complementary areas covered by the chromium plating. Finally, the exposed areas of the original surface are plated with a plating of precious metal, such as gold, silver, platinum, or precious metal alloys.

The process results in a complete decorative design which comprises the chromium plating design and the precious metal plating design.

Chromium is an extremely hard, resistant metal having a color somewhat similar to the color of platinum, and the metal chromium will not tarnish. It may, therefore, be retained in the final decorative design, if desired.

Preferably the precious metal plating has a color which contracts with the chromium plating color. For example, a gold plating, or a green gold plating, may be employed. If desired, the exposed base metal surfaces A', indicated in Fig. 3, may be etched by means of a suitable etching solution, such as ferric chloride, which will not affect the chromium plating. That is, the chromium plating may be used as a resist during the etching operation. Thereafter, the etched base metal areas may be plated with a pre-

cious metal, or precious metal alloy. The chromium plating will not receive the precious metal plating. On the other hand, chromium plating will be received readily by 5 other metals, suitable current density per unit of area being employed in the plating operation.

If desired, after the base plate has received the plating of precious metal, the chromium 10 plating design may be removed, for example, by using dilute hydrochloric acid or dilute sulphuric acid; and the exposed areas of the base plate may then be etched while using the precious metal plating (silver, for example) as a resist. An etching operation 15 of this character is more fully described in the above-mentioned application.

The improved method is applicable to producing decorative designs on various base 20 metals and alloys, such as brasses, bronzes, German silvers, etc.

The foregoing detailed description has been given for clearness of understanding only, and no unnecessary limitations should 25 be understood therefrom, but the appended claims should be construed as broadly as permissible, in view of the prior art.

What I regard as new, and desire to secure by Letters Patent, is:

80 1. The method of treating a base metal surface, which comprises: applying to the surface a suitable resist design; applying a chromium plating design to the exposed areas of the metal surface; removing the resist design, thus leaving areas of the original surface exposed and other areas covered by the chromium plating; etching the exposed areas of the original surface; and plating with precious metal said etched areas while

40 the chromium serves as a resist.

2. A method of treating a base metal surface; which comprises: producing a chromium plating design on a portion of said surface and exposing the remaining areas; 45 and plating said exposed areas with a platable metal of contrasting color, the chromium being used as a resist in the last-mentioned plating operation.

3. A method of treating a base metal surface, which comprises: producing a chromium plating design on a portion of said surface and exposing the remaining areas, and plating said exposed areas with a metal comprising gold while the chromium plating 55 design serves as a resist.

4. The method of treating a metal surface, which comprises: producing a chromium plating design on a portion of said surface and exposing the remaining areas, etching those exposed areas with an etching solution which does not dissolve chromium plate; and plating the etched areas of the original metal while using the remaining chromium plate as a resist.

65 JAMES C. McFARLAND.